

L. R. FERGUSON.

REINFORCED CONCRETE FOR MARINE FOUNDATIONS.

APPLICATION FILED MAR. 8, 1917.

1,285,091.

Patented Nov. 19, 1918.

*Fig. 1.*



*Fig. 2.*



*Fig. 4.*



*Fig. 3.*

Inventor  
Lewis R. Ferguson  
By Alexander S. Bell  
Attorneys

# UNITED STATES PATENT OFFICE.

LEWIS R. FERGUSON, OF PHILADELPHIA, PENNSYLVANIA.

## REINFORCED CONCRETE FOR MARINE FOUNDATIONS.

1,285,091.

Specification of Letters Patent. Patented Nov. 19, 1918.

Application filed March 8, 1917. Serial No. 153,373.

*To all whom it may concern:*

Be it known that I, LEWIS R. FERGUSON, a citizen of the United States, residing at Philadelphia, in the county of Philadelphia, 5 and State of Pennsylvania, have invented certain new and useful Improvements in Reinforced Concrete for Marine Foundations; and I hereby declare that the following is a full, clear, and exact description thereof, 10 reference being had to the accompanying drawings, which form part of this specification.

This invention has particular reference to the construction of partially submerged reinforced concrete foundations for marine work, and has particular reference to reinforced concrete piles, cylinders, columns and the like, used in the construction of docks, wharves, piers and other structures near, in 20 or over salt water. The object of the invention is to enhance the durability of such work, and to protect the same from the action of the damp salt air which has a most destructive effect upon such piles, etc., as 25 heretofore constructed.

It has been known that reinforced concrete piles, cylinders and the like where exposed to the salt water spray and to damp salt air soon crack and spall, such spalling 30 ultimately causing disintegration and failure of the concrete work. This cracking and spalling has heretofore been attributed to causes other than the true one. I have discovered that such cracking and spalling is 35 caused by the rapid corrosion or oxidization of the embedded metal reinforcing. I have also discovered that this cracking always starts above the low water line and is most extensive just above the high water 40 line; that such spalling and cracking follows along the lines of the reinforcing rods, and is usually progressive with the corrosion or rusting of the metal reinforcing. I have discovered that steel or iron reinforcing bars even when embedded in concrete 45 piles to a depth of several inches are rapidly corroded in this way when exposed to damp salt air; and I have further discovered that even when the richest and best made concrete 50 is employed such reinforced piles will crack and spall almost as rapidly as concrete piles of poorer quality. This disintegrating ac-

tion of such reinforced concrete piles is not confined to any particular locality but is prevalent to a more or less marked extent 55 along both the Atlantic and Pacific coasts, and as a consequence all the present reinforced concrete piles exposed as described to sea or salt air are rapidly deteriorating and failing.

I have discovered that if the portion of the metal reinforcing which lies within that portion of the concrete pile, cylinder or column that projects above low water and which is exposed to the action of the damp salt air is formed of or coated, galvanized or plated with tin, zinc or other suitable non 65 corrodible or rust resisting metal or metals that will resist the action of the damp salt air but will not prevent the proper bond or 70 adhesion between the concrete and the metal reinforcing embedded therein; the exposed portions of such reinforced concrete will not be liable to crack and spall and will resist the combined action of the salt air and wash 75 of sea water without deterioration, as well as the submerged portions of the reinforced concrete which are not exposed to the action of air.

I have found that the submerged portions 80 of reinforced concrete piles are not affected and do not crack and spall like the portions of the piles which are above low water; therefore the submerged portion of the concrete structure needs no special treatment.

Heretofore it has been customary to use ordinary black iron or steel bars extending throughout the concrete pile, cylinder or column for reinforcing same; which reinforcing is quickly oxidized by salt air. 90 In carrying out my invention I preferably protect such reinforcing bars, or at least the portions thereof within the upper or exposed portion of the pile; which comes above the low water line, by forming them of a 95 non corrodible metal or galvanizing, tinning, plating or otherwise coating such reinforcement with a non corrodible or rust resisting metal to prevent corrosion of the reinforcement, and by so doing I indefinitely 100 prolong the life of such reinforced concrete piles with negligible additional expense.

I will explain the invention as applied to concrete piles with reference to the accom-

panying drawings which conventionally illustrate a common form of reinforced concrete pile, and the manner of utilizing my invention in connection therewith.

5. In said drawings:

Figure 1 is a side elevation of a reinforced concrete pile.

Fig. 2 is an enlarged sectional view of the upper or exposed part of such pile.

10. Fig. 3 is a transverse section thereof.

Fig. 4 is a view similar to Fig. 2 showing how the upper sections of the reinforcing may be made of a non corrodible metal.

15. The concrete pile 1 may be formed in the usual manner and be of any desired length and cross section; and be provided with any number of reinforcing rods or bars, which may be arranged as usual; four such reinforcing bars 2 being shown in the drawings.

20. These reinforcing bars may be formed of iron or steel, and preferably extend from the lower end to the top of the pile as usual.

25. In carrying out my invention where the reinforcing is of common iron or steel so much of each reinforcing bar 2 as lies within that portion of the pile which will be above low water or exposed to the air when the pile is in position for service is either formed of a noncorrodible metal or galvanized, or 30 plated, or dipped or otherwise coated externally with a metal, such for instance as tin, zinc, copper or an amalgam, to render it non corrosive so that it will resist rust and not be appreciably affected by sea water 35 and salt air.

35. The metallic protective coating 3 may be applied to the bars either by electro-galvanic deposition, dipping in molten metal, or in any other desired and proper manner. Such a coating is indicated at 3 in Figs. 2 and 4 and should be such as will not or cannot separate from the metal reinforcing, and will not prevent the concrete firmly bonding or adhering to the reinforcing when it is cast 45 or molded around the same.

40. The particular form and construction of the concrete piles or foundation members and the specific form or arrangement of the reinforcing members are not essentials of the invention. If desired the protective coating could extend throughout the length of the reinforcing bars, but it is only necessary in practice that such protective coating shall extend over so much of the reinforcing member as is embedded in that portion of the pile which is exposed to the action of the salt air.

45. In some cases the black iron or steel reinforcement may be used in that part of the pile, etc., that will be wholly submerged at low water or when the pile is in position for service as indicated at 2<sup>a</sup> in Fig. 4 and reinforcing sections 2<sup>b</sup> may be spliced or otherwise fastened to the upper ends of 50 bars 2<sup>a</sup> and extend in the exposed portion of

the pile above low water; such sections 2<sup>b</sup> being either formed of or coated with a rust resisting metal.

55. This invention applies to the precast as well as the cast in place type of reinforced concrete pile and the like. It also applies to reinforced concrete cylinders and the like where wholly cast in place, or made by pre-casting a reinforced concrete shell several inches or more in thickness and thereafter filling such shell with concrete after the shell is in position. It also applies to other forms of reinforced concrete foundation members used in marine construction.

60. What I claim is:

1. A reinforced concrete member partly submerged in sea water and comprising a concrete body and metal reinforcement embedded therein, and having a part of said reinforcement within the portion of the member exposed to the atmosphere when *in situ* rust-resisting to prevent spalling of the concrete.

2. A reinforced concrete body, partly submerged in sea water, having metal reinforcing members therein extending below the water line; the parts of the reinforcing members in the portion of the body exposed to the atmosphere when *in situ* being non corrodible to prevent spalling or disintegration of the concrete.

3. A reinforced concrete member partly submerged in sea water and comprising a concrete body and a metal reinforcement embedded therein, the parts of said reinforcement within the portion of the member exposed to the atmosphere when *in situ* being protected by a rust-resisting metallic coating to prevent spalling of the concrete.

4. A concrete foundation member to be partly submerged in sea water and comprising a concrete body and metal reinforcing bars embedded therein, said reinforcing bars in the portion of the member above low water and exposed to the atmosphere being protected by rust-resisting metallic coating to prevent spalling of the concrete.

5. A concrete foundation adapted to be partly submerged in sea water comprising a concrete body, and a plurality of metal reinforcing bars therein, the parts of the bars within the portion of the body which is exposed to the atmosphere when *in situ* having a rust-resisting metallic coating applied thereto prior to being embedded in the body to prevent spalling of the concrete.

6. A pile adapted to be partly submerged in sea water, comprising a concrete body and a plurality of metal reinforcing members embedded therein; and having the parts of said members in the portions of the pile exposed to the atmosphere when *in situ* rust-resisting to prevent spalling of the concrete.

7. A concrete pile adapted to be partly

submerged in sea water, having longitudinally disposed metal reinforcing members embedded therein, the parts of said members in the portions of the pile which will be exposed to the atmosphere when *in situ* being rust-resisting to prevent spalling of the concrete.

8. A pile adapted to be partly submerged in sea water, comprising a concrete body, and metal reinforcing members embedded in and extending longitudinally of the pile, the parts of said members in the portions of the pile exposed to the atmosphere when *in situ* being formed of a rust-resisting metal, substantially as and for the purpose specified.

9. A pile adapted to be partly submerged in sea water, comprising a concrete body, and a plurality of metal reinforcing bars embedded in and extending longitudinally of the pile, the parts of said bars in the portions of the pile exposed to the atmosphere when *in situ* having a metallic rust-resisting coating applied to their outer surfaces prior to fabrication in the pile, substantially as described.

10. The method of protecting reinforced concrete partly submerged in sea water and comprising a concrete body with metal reinforcement embedded therein; consisting in making the part of said reinforcement with-

in the portion of the concrete exposed to the atmosphere rust-resisting to prevent spalling of the concrete.

11. The method of protecting reinforced concrete partly submerged in sea water, and comprising a concrete body and metal reinforcement embedded therein; consisting in coating the parts of said reinforcement within the portion of the concrete body exposed to the atmosphere with rust-resisting material to prevent spalling of the concrete.

12. The method of protecting reinforced concrete adapted to be partly submerged in sea water and comprising a concrete body and metal reinforcement embedded therein; consisting in providing the parts of said reinforcement in the portions of the concrete exposed to the atmosphere with a rust-resisting coating to prevent spalling of the concrete.

13. The method of protecting reinforced concrete adapted to be partly submerged in sea water and comprising a concrete body and reinforcement embedded therein; consisting in making the parts of said reinforcement in the portion of the concrete exposed to the atmosphere of rust-resisting metal to prevent spalling of the concrete.

In testimony that I claim the foregoing as my own, I affix my signature.

LEWIS R. FERGUSON.